

# UNITED STATES PATENT OFFICE.

HENRY GERNER, OF NEW YORK, N. Y., ASSIGNOR TO THE HEVEENOID  
MANUFACTURING COMPANY, OF SAME PLACE.

## PROCESS FOR THE TREATMENT OF INDIA-RUBBER, &c.

SPECIFICATION forming part of Letters Patent No. 226,057, dated March 30, 1880.

Application filed March 5, 1880. (No model.)

*To all whom it may concern:*

Be it known that I, HENRY GERNER, of the city, county, and State of New York, have invented a new and useful Process in the 5 Treatment of India-Rubber, Gutta-Percha, and Analogous Gums, which process is fully set forth in the following specification.

The object of my invention is to purify more thoroughly, and in a cheaper and more expeditious manner than heretofore done, india-rubber, gutta-percha, and analogous gums, and to convert the same into a more homogeneous mass, free from impurities, air, and moisture, with which mass is more readily and 10 more thoroughly incorporated free sulphur, or sulphur in its various chemical combinations, as also pigments, colors, and all the different substances and ingredients with which such gums are generally mixed, or with which they 15 may be mixed, for different manufacturing purposes.

The imported gum is always impure, owing to the mode of gathering and drying employed, and is often purposely adulterated with clay, 20 leaves, sand, bark, and the like. It is necessary that these impurities and adulterations should be removed before the gums can be adjudged to be in a fit state to be converted 25 into the numerous articles of industry and commerce for which they are and can be employed. The more thoroughly this purification is effected the better, more satisfactory, and 30 more valuable will be the articles produced.

At present the imported gum is usually cut 35 into thin shreds or minced into small parts and washed by agitation in warm water, after which it is dried. The fragments are then brought between iron rollers under a stream of water, and thus receive a second purification 40 at the same time that the several parts are rolled together into one sheet. If foreign substances are still contained in the gum, the sheet is returned to a hopper over the rollers and passed repeatedly between them. After this 45 cleansing and treatment the gum is kneaded on another machine, called the "mill," for the purposes of expelling air and moisture and giving it greater density. That the power to work this mill is very great is evident from

the fact that if the drum of the mill is less 50 than three inches in diameter it is twisted asunder, and heat is evolved during the operation to such an extent that the stream of cold water used to wash the gum is brought very rapidly to a boiling-point, and if cold 55 water is not constantly supplied the temperature rises to such a height that the mass cannot be touched by the hand. After this the gum is further subjected to treatment in another machine, somewhat of the same construction 60 as the foregoing, wherein the water and air taken up in the mill are caused to be expelled. The gum, after all these manipulations, is still not yet sufficiently dense for its various uses. To obtain the required density the gum, 65 in the form of balls, is introduced into a larger cylinder, where it gets incorporated into one mass, which is compressed in cast-iron molds by aid of powerful presses, and kept in this compressed state for several days. 70

This costly and unsatisfactory process is of all known methods up to the present time still carried out as the best, and is the method now pursued in the principal European and American india-rubber factories; and it may be 75 readily inferred how important must be a less complicated and more satisfactory process which will accomplish the end sought for, and which may be taken advantage of by following the directions I am about to set forth, to 80 enable others to make and use my invention.

I take the imported raw gum as it occurs in commerce, and subject it to a washing in a tub or drum or other suitable vessel, as may be desired. I prefer to use warm water at, say, 85 a temperature of 90° to 100° Fahrenheit, in which a handful of soda, to produce a quicker and better result, may be dissolved in, say, every fifty gallons of water. When, by this process, the outside dirt is removed, I cut the 90 gum, on a suitable machine or machines, into minute parts—say of the size of grains. I then spread this minced gum on flat troughs, which I place on shelves in a suitably-constructed ice-house, where the gum is frozen to 95 a temperature below zero, or at least below the Fahrenheit freezing-point of water, when it becomes hard and brittle, losing its elas-

ticity, and appearing more opaque than when it is heated or when in its natural state under normal temperatures. In this frozen state the gum is brought onto a suitably-constructed mill, which is so constructed that ice can be lodged in its interior parts, by means of which the grinding-surfaces of the mill are kept as cold as the frozen gum. In this mill the gum is rapidly and readily converted into very minute parts, like those of flour or fine powder.

It is evident that any substance which will freeze the gum and cool the mill may be employed instead of the natural ice described.

When the ground gum leaves the mill it drops down into a suitably-constructed receptacle partly filled with cold water, in which the gum is agitated until it has parted with all foreign substances. The gum is now dried by suitable means until all moisture is expelled, and is then, in a close vessel, exposed to the action of any suitable solvent, such as bisulphide of carbon, gasoline, or other of a like nature, by aid of which it is converted into a pasty or fluid state, as may be required, according to the different purposes for which it may be employed.

The greater part of the solvent used may be recovered for reuse after having served its purpose of dissolving the gum and bringing it into a homogeneous mass by constructing the metallic vessel in which the process of solution is conducted with a surrounding jacket, into which steam is conducted, which serves to heat the vessel and distill off the solvent through a suitably-constructed and cooled worm or condenser connected with the vessel itself; and through this condenser it is distilled off into a closed receiver, in which it is

kept for use for dissolving purposes over and over again. The dissolved homogeneous mass is then removed from the solution-vessel and placed into a suitable mixing and kneading machine, where it is mixed with the required substances either for curing, vulcanization, or incorporation with pigments or colors, or for giving body and bestowing other properties, as may be required for different purposes of manufacture and use. After the thorough incorporation of the gum with these substances it is rolled, molded, formed, or pressed into all manner of required forms or shapes, either alone or in combination with textile fabrics or fabric and goods of any description. The curing or vulcanization of the gum may then be proceeded with by any of the well-known used methods.

Having thus fully described my invention, I desire to claim—

1. In a process for treating india-rubber, gutta-percha, or other like gums, the freezing and grinding of the same, as set forth.

2. The herein-described process of treating india-rubber or similar gums, consisting of first washing in warm water in which is dissolved some soda, then cutting it into small particles, then freezing, then grinding in a frigid mill, again washing in cold water, then subjecting to the action of solvents in a closed vessel, and finally mixing with any desired substance, and manufactured or used in the common ways, substantially as set forth.

HENRY GERNER.

Witnesses:

RICHARD GERNER,  
M. DITTEHOFER.